

June 14, 1960

G. F. DAVIES

2,940,163

ALLOY CLAD TITANIUM AND METHOD OF PRODUCING SAME

Filed Aug. 5, 1954



FIG. 1



FIG. 2



FIG. 3



FIG. 4

INVENTOR.

GAIL F. DAVIES

BY

*Max L. Raymond*

AGENT

1

2,940,163

## ALLOY CLAD TITANIUM AND METHOD OF PRODUCING SAME

Gail F. Davies, Willoughby, Ohio, assignor to Clevite Corporation, Cleveland, Ohio, a corporation of Ohio

Filed Aug. 5, 1954, Ser. No. 448,106

15 Claims. (Cl. 29—182.2)

This invention relates broadly to a process for the production of a titanium alloy-clad titanium article and to the article of manufacture produced thereby.

The invention relates more specifically to the novel process for the production of a titanium alloy-clad titanium article by powder metallurgy techniques.

An important object of this invention is the production of a novel composite article of titanium and a titanium alloy having therebetween a bond which is highly resistant to shear and tensile separation.

A further object of this invention is the production of an alloy clad relatively light weight titanium article which may be used as armor plate, for rocket nozzle lining, in high wear applications such as gears, impellers, etc., and for chemical apparatus subjected to corrosive atmosphere.

Other objects and advantages will become apparent as the description proceeds.

Referring to the drawing:

Figure 1 is a vertical sectional view of apparatus for practicing the invention, viz., a sintering furnace and press showing the positioning of the die and the metal powders therein.

Figure 2 is a cross-sectional view of an alloy-clad titanium bar according to the present invention showing the bond between the alloy and the titanium metal.

Figures 3 and 4 represent a cross-sectional view of a powder charge prior to applying heat and pressure showing an example of indentations that may be made in the initial powder layer for altering shear and tensile characteristics of the bond.

While unalloyed titanium metal possesses certain distinctive and advantageous metallurgical characteristics, alloys of titanium are likewise found to have many valuable properties. In combining a layer of titanium metal with a layer of an alloy of titanium in accordance with the present invention there are found to be advantages resulting not possessed by either titanium or titanium alloy alone.

One main difficulty in producing a composite structure of titanium metal and titanium alloy is the elimination of exfoliation at the bond between the titanium and titanium alloy and the production of a bond highly resistant to shear and tensile separation.

It has been discovered that such a bond may be produced between titanium metal and titanium alloys using powder metallurgy techniques wherein titanium and titanium alloy powder layers are compressed and sintered together in a die to form a composite article of titanium and titanium alloy joined by a bond having a monotonic compositional gradient across its thickness ranging from substantially unalloyed titanium at one surface to the titanium alloy at the other.

Referring to Figure 1, showing one embodiment of the invention, an amount of titanium powder based on the finished thickness of the titanium layer desired is placed in a die generally shown as 3 made of a suitable material such as graphite positioned within a furnace

2

generally shown as 6, having a gas tight cover 7 and heating means such as a resistance coil 8 surrounding the graphite die. Other conventional heating means may be employed such as a hydrocarbon burner or electrical induction. The resistance coil terminals are connected to terminals outside of the furnace through gas tight insulators 9 and 10. The plunger 2 is connected to an external prime mover by rod 11 which passes through a gas tight gland 12 in top 7. The interior of the furnace 10 may be evacuated through exit 13 by connecting same to a vacuum pump. The titanium charge is leveled and a slight pressure is applied by plunger 2 to pack the surface and prevent random sifting of one powder into the other. The plunger is removed from the die and an overlay charge of titanium alloy powder or intimately mixed titanium and alloying metal powders 4 is introduced and leveled. A vacuum or inert atmosphere is produced in the die cavity. Heat is applied to the die cavity from an external source and pressure is applied by means of plunger 2. The powders are subjected to a temperature from 600 to 1350° C. and pressures from 300 to 1500 p.s.i., depending upon the alloy used, for a period of time sufficient to effect controlled interdiffusion of the titanium metal and the alloy so as to form a graduated bond whose edges are substantially parallel to the original interface between the titanium and titanium alloy powders. The interdiffusion is found to be in a direction substantially normal to the interface, the extent of interdiffusion depending upon the alloy, the temperature, the pressure and the length of time the particular conditions of temperature and pressure are applied. The alloying powder may be in the form of alloy powder, titanium powder coated with alloying metals or a mixture of titanium and alloying metal powders.

Figure 2 represents a cross-sectional view of a finished bar showing the titanium metal layer 1 with the titanium alloy overlaying 4 and graduated bond 5 therebetween. The term graduated bond is intended to define the laminar zone of interdiffusion intermediate the substantially pure titanium metal and the titanium alloy. The composition of the bonding layer progresses from pure titanium metal to the alloy composition in a uniform gradient so that no definite line of demarcation exists between the titanium alloy, the bond, and the titanium metal.

The initial charge of titanium powder may have indentations 14, 15 pressed into the upper surface thereof, as illustrated in Figures 3 and 4, to produce a predetermined configuration in the graduated bond. This may be designed to more evenly distribute shear and tensile stress.

In some instances an advantage may be obtained by depositing an alloy powder of intermediate composition between the titanium metal powder and the alloy powder overlay. With this technique closer control over the rate of diffusion may be accomplished.

Alternate layers of titanium and alloy powders may be charged into the die to produce a laminated product. Preferably the titanium metal powder should be as free as practically possible from oxygen, hydrogen and nitrogen contamination to avoid undue embrittlement of the titanium metal.

Where the alloy has a eutectic having a melting point lower than the sintering temperature such that a liquid phase may exist, the alloy powder should be placed below the titanium powder to avoid too rapid or spotty penetration by the alloy as a result of the action of gravity.

A specific application of this novel process to the production of titanium alloy clad titanium plate for use as armor comprises using an alloy powder comprising 95% titanium, 2% iron and 3% aluminum. The titanium and alloy powders in predetermined amounts are

respectively charged into the die and heated from 600 to 1350° C. under pressure from 300 to 1500 p.s.i. for about 2 to 8 hours depending upon the thickness of the graduated bond desired. When completed the plate is allowed to cool in the die and then removed from the die. The alloy side of the plate is hard and somewhat brittle while the titanium remains ductile. When used as armor plate with the alloy side outermost, the hard alloy tends to shatter or retard the projectile on impact while the ductile titanium backing absorbs the shock and prevents fissures, developed in the alloy as a result of the impact, from penetrating the plate. Better impact and penetration resistances are obtained on tests of this armor plate than in any known armor of comparable weight and thickness. Other alloys which are useful for producing armor are RC130B titanium alloy containing 3.5-4.5% Mn, 1-2.5% Fe, 3.5-4.5% Al and the balance substantially titanium; RC150A titanium alloy containing 1.3% Fe, 2.5% Cr and the balance substantially titanium; and titanium manganese complex alloy containing 3% Mn, 1% Al, 1% V, 1% Cr, 1% Fe and the balance substantially titanium.

An example of the application of this invention to the production of high temperature and flame erosion resistant alloy clad titanium for use as rocket nozzles and the like comprises using an alloy powder selected from titanium ceramets such as titanium-titanium boride, titanium-titanium carbide, titanium-titanium silicide and aluminum alpha and gamma stabilized alloys of titanium. The alloys may be introduced into the die as alloy powders or they may be formed in situ by introducing a mixture of the powders making up the alloy. A layer of titanium powder and a layer of titanium alloy powders are placed in the die and heated from 600 to 1350° C. under from 300 to 1500 p.s.i. for a period of time sufficient to produce a graduated bond. The finished article has a refractory like surface capable of withstanding high temperatures and flame erosion encountered in high temperature applications such as rocket nozzles while the ductile titanium backing provides the necessary structural strength and shock resistance needed to prevent failure under severe conditions of temperature and acceleration.

A further application of this invention comprises the production of a titanium article having an alloy cladding characterized by high wear resistance, such as high oxygen content titanium containing from 1-4% O<sub>2</sub> and high nitrogen content titanium alloy. Such articles may be used as gears, bearing surfaces and the like, where high wear is encountered. The hard alloy surface may be ground to a super finish and the property of hardness plus the unusual surface smoothness results in low friction losses and the high wear resistance.

Alloys which have been successfully bonded to titanium by this process to form alloy clad titanium are RC130B titanium alloy containing 3.5-4.5% Mn, 1-2.5% Fe, 3.5-4.5% Al and the balance substantially titanium; titanium-manganese complex alloy containing 3% Mn, 1% Al, 1% V, 1% Cr, 1% Fe and the balance substantially titanium; high oxygen titanium containing from 1-4% O<sub>2</sub>; 150A titanium alloy containing 1.3% Fe, 2.5% Cr and the balance substantially titanium; titanium-titanium carbide alloys containing approximately 20-75% Ti and the balance 80-25% TiC; titanium-titanium boride alloys, one containing approximately 10% TiB and the balance Ti and the other containing approximately 10% TiB<sub>2</sub> and the balance Ti; titanium-aluminum alloys containing about 12% Al (alpha stabilized) and high aluminum titanium base alloys containing about 36% Al (gamma stabilized).

While this invention has been described and illustrated by the example shown it is not intended to be limited thereto and other modifications may be employed within the scope of the following claims.

We claim:

1. The method of producing alloy-clad titanium comprising: compacting and sintering together along an interface respective masses of titanium powder and a titanium alloy powder under a pressure of from about 300 to 1500 p.s.i. while heated to a temperature of from about 600° to 1350° C. in a substantially inert atmosphere for a sufficient period of time, not less than 15 minutes, to produce a bond between said masses comprising a laminar zone of interdiffused titanium and titanium alloy at said interface, said zone having a uniform compositional gradient in its thickness direction ranging from essentially unalloyed titanium at the surface of said zone adjacent the titanium mass to said titanium alloy at the opposite surface of said zone.

2. The method of producing alloy-clad titanium comprising compacting and sintering together along an interface superimposed masses of titanium powder and an alloy powder selected from the group consisting of (1) a mixture of titanium powder and an alloying metal powder and (2) titanium alloy powder under a pressure of from about 300 to 1500 p.s.i. while heated to a temperature of from about 600° to 1350° C. in a substantially inert atmosphere for a sufficient period of time, not less than 15 minutes, to produce a bond between said masses comprising a laminar zone of interdiffused titanium and titanium alloy at said interface, said zone having a uniform compositional gradient in its thickness direction ranging from essentially unalloyed titanium at the surface of said zone adjacent the titanium mass to said titanium alloy at the opposite surface of said zone.

3. The method of producing alloy-clad titanium comprising: placing in a suitable die a charge of finely divided titanium powder; leveling and applying a slight press to the charge; placing in said die, superimposed on said charge, a second charge of metal powder selected from the group consisting of (1) a mixture of titanium powder and alloying metal powder and (2) titanium alloy powder; producing a vacuum in the die cavity; heating the die charges to a temperature from about 600° to 1350° C. while applying thereto a pressure in the range from about 300 to 1500 p.s.i.; and maintaining said temperature and pressure for a sufficient period of time, not less than 15 minutes, to produce a bond between said masses comprising a laminar zone of interdiffused titanium and titanium alloy at said interface, said zone having a uniform compositional gradient in its thickness direction ranging from essentially unalloyed titanium at the surface of said zone adjacent the titanium mass to said titanium alloy at the opposite surface of said zone.

4. A composite metal structure consisting of sintered titanium metal backing and a sintered titanium alloy cladding bonded to said backing by a laminar zone of interdiffusion at the interface between the backing and cladding, said laminar zone having a compositional gradient in the thickness direction, the end components of said gradient being substantially unalloyed titanium adjacent the backing and said titanium alloy adjacent the cladding.

5. A composite armor plate consisting of a ductile sintered titanium metal basis clad with brittle sintered titanium alloy bonded to the basis by a laminar zone of interdiffusion at the interface between the basis and cladding, said laminar zone having a monotonic compositional gradient in the direction of its thickness, the composition at the respective ends of said gradient conforming substantially to that of the basis and cladding, respectively.

6. A composite armor plate according to claim 5 wherein said titanium alloy is an Fe-Al titanium alloy.

7. A composite metal structure consisting of a mass of essentially unalloyed ductile sintered titanium and a mass of a sintered titanium alloy bonded together by a laminar zone of interdiffusion at the interface between said masses, said laminar zone having a monotonic com-

75

positional gradient in the direction of its thickness, the composition at the respective ends of said gradient conforming substantially to that of the respectively contiguous mass.

8. A composite metal structure according to claim 7 wherein said titanium alloy is a heat resistant titanium cermet alloy selected from the group consisting of titanium-titanium boride; titanium-titanium carbide; and titanium-titanium silicide.

9. A composite metal structure according to claim 7 wherein said alloy is an aluminum alpha stabilized titanium alloy.

10. A composite metal structure according to claim 7 wherein said alloy is 2% Fe, 3% Al titanium alloy.

11. A composite metal structure according to claim 7 wherein said alloy is an aluminum gamma stabilized titanium alloy.

12. A composite metal structure according to claim 7 wherein said alloy is a titanium-oxygen alloy.

13. A composite metal structure according to claim 7 wherein said alloy consists essentially of from 25 to 80% titanium carbide and the balance titanium.

14. A composite metal structure according to claim 7 wherein said alloy is a titanium-titanium nitride alloy.

15. The method of producing an alloy clad titanium composite comprising: superimposing separate layers of 5 titanium powder and a titanium alloy powder consisting essentially of powdered titanium and at least one alloy forming element in alloying amounts selected from the group consisting of carbon, boron and silicon; pressing said layers together under a pressure of from about 300 p.s.i. to about 1500 p.s.i.; and heating the layers to a temperature of from about 600° C. to about 1350° C. in an inert atmosphere for at least 15 minutes to produce interdiffusion of metal between the two layers.

References Cited in the file of this patent

UNITED STATES PATENTS

|           |           |               |
|-----------|-----------|---------------|
| 2,491,284 | Sears     | Dec. 13, 1949 |
| 2,674,542 | Alexander | Apr. 6, 1954  |
| 2,703,750 | Cotter    | Mar. 8, 1955  |